

Jan. 22, 1929.

1,699,704

A. L. H. LEDEBOER

FIBER SPOOL AND PROCESS

Filed Jan. 4, 1927

3 Sheets-Sheet 1

F I G . 1 .



F I G . 2 .



F I G . 3 .



F I G . 4 .



F I G . 5 .



F I G . 6 .



INVENTOR  
Adrian L. H. Leedeboer.  
BY *White & Post.*  
his ATTORNEYS

Jan. 22, 1929.

1,699,704

A. L. H. LEDEBOER

FIBER SPOOL AND PROCESS

Filed Jan. 4, 1927

3 Sheets-Sheet 2

FIG. 7

FIG. 8



FIG. 9



FIG. 10

INVENTOR  
Adrian L. H. Ledeboer  
BY  
White & Pirst  
his ATTORNEYS

Jan. 22, 1929.

1,699,704

A. L. H. LEDEBOER

FIBER SPOOL AND PROCESS

Filed Jan. 4, 1927

3 Sheets-Sheet 3

FIG. 11.

FIG. 12.



FIG. 13.



INVENTOR  
Adrian L. H. Leedeboer  
BY  
White & Post.  
his ATTORNEYS

## UNITED STATES PATENT OFFICE.

ADRIAN L. H. LEDEBOER, OF SAN FRANCISCO, CALIFORNIA, ASSIGNOR TO CHARLES H. SMITH, OF PAWTUCKET, RHODE ISLAND.

## FIBER SPOOL AND PROCESS.

Application filed January 4, 1927. Serial No. 158,937.

This invention relates generally to a spool of novel construction and process of making the same.

Large quantities of spools are consumed 5 annually in the sale of thread, yarns, ribbons and other such goods. These spools are at present being manufactured from soft white woods by the use of automatic wood turning lathes. While wooden spools have proven 10 satisfactory, suitable wood for their manufacture is becoming scarce in this country, and a continued increase in the cost of production is inevitable. Furthermore, wood turning lathes are expensive to maintain and 15 operate and a large percentage of the raw material is necessarily wasted.

It is an object of this invention to devise a spool which may be manufactured from cheap raw material without the use of wood 20 turning lathes.

It is a further object of this invention to devise a strong durable composite spool of fibrous material.

It is a further object of this invention to 25 devise a spool of homogeneous material containing fiber felted in such a manner as to provide strong and durable end flanges.

It is another object of this invention to devise a novel process for manufacturing a 30 spool of fibrous material.

Further objects of this invention will appear from the following description in which I have set forth the preferred embodiment of my invention. It is to be understood that the 35 appended claims are to be accorded a range of equivalents consistent with the state of the prior art.

Referring to the drawings:

Figs. 1 to 4 inclusive illustrate various 0 forms assumed by the fibrous material in the manufacture of the spool.

Fig. 5 is a perspective view of a finished spool made in accordance with this invention.

Fig. 6 is a cross sectional view taken 5 through the spool shown in Fig. 5.

Figs. 7 to 9 inclusive illustrate the steps 0 of the process necessary to form the fibrous material into the shapes shown in Figs. 1 to 4 inclusive.

Fig. 10 is a side elevational view in cross section showing the final step in the process of forming the blank shown in Fig. 4.

Figs. 11, 12 and 13 illustrate the steps of

forming a spool out of the blank shown in 55 Fig. 4.

The distinguishing characteristics of the spool of this invention may be best understood by first describing the process of manufacture. The material which I prefer to employ is 60 cellulose fiber, commonly known as wood pulp or paper pulp. This material not only has the requisite properties for the production of a high grade composite spool, but is also a 65 relatively cheap material since it may be made from low grade woods or other vegetable fibers. If the cellulose pulp is colored because of the nature of the wood or vegetable fiber from which it is manufactured, it is 70 preferably bleached so that the final spool 75 will be white in color. A mass of this cellulose fiber is subjected to pressure in suitable dies, the material being initially in a plastic state as by mixing the same with water. For example, a mass having proper plasticity 75 may have the proportions of one or more grains of pulp to one cubic inch of water. If a definite amount of pulp is employed for forming a given size of spool, the hardness 80 of the spool may be controlled by varying the 85 percentage of pulp in the water.

In Fig. 1 the mass 10 represents a certain volume of plastic cellulose pulp which is introduced into dies to form the mass 11 shown in Fig. 2. Referring to Figs. 7 and 8 a suitable apparatus for treating the cellulose pulp is diagrammatically illustrated as comprising movable dies 12 and 13 having opposed curved faces 15 and 16, the dies being preferably heated. The plastic mass 10 is first positioned in a pocket 18 and is then forced as by means of plunger 19 into the space between dies 13 and 14. A core or pin 21 is provided intermediate the dies so as to form a central passageway through the pulp mass. Pressure is then applied to the dies 12 and 13 to 90 form the mass into the shape shown in Figs. 9 and 10. The water or other liquid squeezed from the mass during this operation may be removed through the hollow dies which are 95 shown as provided with perforations 22 and 23 for this purpose. It will be noted that this pressure is applied lateral to, or at right angles to the axis of pin 21. When pressure is applied to cellulose pulp, the fiber tends to 100 arrange itself in directions substantially normal to the direction of the applied force. Therefore, as shown in Fig. 10, the fiber 24

of the pulp mass arranges itself in the general direction of the pin 21, and also becomes felted or interlocked together.

In Figs. 3 and 4 there is shown a blank 26 of cylindrical shape having a central passageway 27, which blank is formed after the dies 12 and 13 are closed to the position shown in Figs. 9 and 10. As previously explained, the fiber 24 of this blank have been felted together and are arranged in the general direction of the axis of passageway 27. This blank is then placed between another set of heated dies 28 and 29 which have their faces formed to provide the spool flanges. Thus the die 15 faces 31 and 32 are provided with end pockets 33 and 34, which when the dies are in closed position form flanges of the desired size upon the spool ends. To maintain the passageway 27, a pin 36 is extended through the blank 20 and the dies are then moved to the closed position shown in Fig. 12. The intermediate portion of the pulp mass is thus further compressed and the pockets 33 and 34 are filled to form the spool flanges. During this step of 25 the process the fiber 37 constituting the flanges arrange themselves at an angle to the spool axis, because the fiber near the ends of blank 26 tends to remain substantially parallel to the deformed surfaces forming the 30 inner faces of the flanges. However, to further strengthen the spool flanges, plungers 38 and 39 are provided to press against the spool ends. As shown in Fig. 13 when dies 28 and 29 have been moved to closed position 35 plungers 38 and 39 are forced inwardly to compress the fiber in the spool ends. This pressure provides a layer of felted fiber 41 lying in a general direction parallel to the planes of the spool ends, which serve to reinforce the flanges.

The finished spool is shown in Figs. 5 and 6, the cross section of Fig. 6 showing the intermediate fiber 42 arranged substantially parallel to the spool axis and the end fiber 45 41 arranged at an angle to the axis or substantially in the direction of the plane of the spool ends. It is likewise characteristic of the product that the fiber of the surface layer is practically all arranged parallel to the adjacent surface, and is felted in such a manner 50 as to reinforce the spool against all possible stresses. If desired, one or both plungers 38 and 39 may be provided with raised or depressed letters or other marks for stamping 55 upon the spool ends.

It is obvious that various chemicals can be mixed with the pulp to increase its hardness and durability. Such chemicals are introduced and thoroughly mixed with the pulp 60 before introduction into the dies. For example, the mixture of pulp, water and chemical may be thoroughly mixed in a vat by mechanical agitators. Care should be taken to introduce no chemicals which might discolor 65 the spool or which may injure the thread or

other goods to be wound upon the same. Examples of binders which may be used to add to the hardness of the spool are starch, glues, solutions of sodium or potassium silicate, and these substances may be used with such fillers 70 as magnesia, borax, talcum, lime or other such material. Suitable sizes may also be employed if a smoother surface is desired. Instead of premixing the chemical with the pulp and water, it may be introduced into the 75 pulp mass while in the dies. For example, pin 21 may be made hollow and perforated so that chemicals introduced into this pin or tube will be injected into the pulp mass.

The product of this invention has all the 80 desirable characteristics of wooden spools, and has the additional advantage of being manufactured from a cheap inexhaustible supply of raw material. Furthermore, the process of manufacture is readily adaptable 85 to automatic machinery, which is cheap to maintain and requires a minimum of skilled labor for its operation.

I claim:

1. An article of manufacture comprising 9 a spool made of a homogeneous integral mass containing felted fiber, the fiber of the intermediate portion of the spool extending in the same general direction as the spool axis.

2. An article of manufacture comprising a 9 spool made of a homogeneous integral mass containing felted fiber, the fiber in the intermediate portion of the spool extending in the same general direction as the spool axis, and the fibers in the spool flanges lying at an angle 1 to the spool axis.

3. An article of manufacture comprising a spool made of a homogeneous integral mass containing felted fiber, the fiber in the intermediate portion of the spool extending in the 1 same general direction as the spool axis, and the fibers in the spool flanges extending in the same general direction as the planes of the spool ends.

4. In a process of making a spool of fibrous 1 material, the steps of forming a felted blank of the material, and then compressing the blank laterally to form the shape of a finished spool.

5. In a process of making a spool of fibrous 1 material, the steps of forming a cylindrical blank of the material, and then compressing the blank laterally to form the shape of a finished spool.

6. In a process of making a spool of fibrous 1 material, the steps of forming a felted blank of the material with an axial passage, and then compressing the blank laterally to form the shape of a finished spool.

7. In a process of making a spool of fibrous 1 material, the steps of applying lateral pressure to a plastic mass of the material to cause the fiber to arrange itself substantially normal to the direction of force and applying pressure to the ends of the mass to arrange 1

the fibers adjacent the spool ends in a direction substantially normal to the spool axis.

8. In a process of making a spool of fibrous material, the steps of applying pressure at opposite ends of a fibrous mass to arrange the fibers adjacent the spool ends at an angle to the spool axis, and applying lateral pressure to the mass to felt the fiber in the intermediate portion of the spool.

10. In a process of making a spool of fibrous material comprising forming a felted blank of the material by lateral pressure to a plastic mass of the fiber, shaping the blank into a

spool by pressure, and applying pressure to the ends of the spool. 15

10. An article of manufacture comprising a spool made of a homogeneous mass consisting principally of felted cellulose fiber, the fiber in the intermediate portion of the spool extending in the same general direction as the spool axis and the fiber of the spool flanges extending in the same general direction as the planes of the spool ends. 20

In testimony whereof, I have hereunto set my hand.

ADRIAN L. H. LEDEBOER.